

## UNITED STATES PATENT OFFICE

2,376,306

## MINERAL OIL COMPOSITION

John H. Bishop, Wenonah, N. J., assignor to  
 Socony-Vacuum Oil Company, Incorporated,  
 New York, N. Y., a corporation of New York

No Drawing. Application March 17, 1942,  
 Serial No. 435,077

6 Claims. (Cl. 252—47)

This invention has to do with lubricants and is more particularly concerned with lubricants for ferrous metal surfaces in an environment where such surfaces are also subject to contact with water and in consequence are likely to rust.

As is well known to those familiar with the art, difficulties have been experienced during the operation of steam turbines, and particularly during the initial operation of new steam turbines, because of the rusting of ferrous metal parts. The combination of fresh (not previously used) oil; clean, new metal surfaces; and moist conditions of operation of new steam turbines appears particularly conducive to rusting difficulties. Particles of rust formed on or carried to the bearing surfaces of small clearance, such as the governor, for example, tend to cause sticking, which renders them inoperative. In cases of severe rusting, bearings may be injured.

This rusting phenomenon under conditions or the type outlined above is evidently the result of improper or inadequate "wetting" of the metal surfaces with oil, thus permitting a preferential contact of the surfaces with the water which is present. One expedient used in the past to prevent rusting under these conditions has been to mix with the new oil several per cent of an oil which has been previously used in turbine operation for a considerable period of time. The oxidation products in the used oil cause the oil to "wet" more adequately and better adhere to the metal surfaces. Such an expedient, however, not only introduces those oxidation products which protect against rusting but introduces as well other oxidation products, which promote the formation of sludge and acidity, and increase emulsifying tendencies. Other materials such as stearic acid have been proposed; but such additives, although they do prevent rusting, have the undesirable property of unduly raising the acidity (neutralization number, or N. N.) of the oil and of accelerating the development of acidity in use.

The present invention is predicated upon the discovery that the admixture with a viscous mineral oil, such as a turbine oil or the like, of minor proportions of both an aniline disulphide and degras (wool grease) fatty acids provides an oil composition of improved properties. For example, such oil compositions when used in steam turbines, particularly during the break-in period of a new turbine, will cause a preferential wetting of the metal surfaces with the oil and will prevent undue rusting of the metal parts. This new and novel combination of improving agents in a turbine oil functions in several ways in that it adequately "wets" the metal surfaces, and inhibits the deleterious effects of oxidation upon the oil. The incorporation of from about

0.05% to about 0.2% of an aniline disulphide, and from about 0.01% to about 0.1% of degras fatty acids, in a turbine oil will not only prevent undue rusting of the metal parts of a new turbine, especially during the break-in period of a new turbine, when such problem is most acute, but will, in addition, increase the effective life of the oil composition.

I am aware of the fact that it has been proposed, in U. S. Patent No. 2,151,353, to use degras fatty acids in relatively large proportions of from 5% to 20% in coating and drawing compositions. The present invention distinguishes over the aforesaid disclosure in the discovery that with the combination contemplated herein, a very small quantity—of the order of 0.10% or less—of degras fatty acids may be used to improve turbine oils.

When large quantities, such as 5% to 20% (as disclosed in the aforesaid patent), of degras fatty acids are used in turbine oils substantial and undesirable emulsification of the oil is caused. I have found, however, that when not more than 0.10% of degras fatty acids is used in combination with a minor proportion of an aniline disulphide in turbine oils, the emulsification tendencies of the oil composition are substantially reduced, so much so, in fact, that the compositions contemplated herein are extremely effective and desirable for use in turbines. As small a quantity as 0.01% of the degras fatty acids may be used in the turbine oil compositions contemplated herein to obtain improvement in rust prevention and effective life of the oil. Thus, it will be seen that the quantity of degras fatty acids which can be used in the turbine oil compositions contemplated herein is determined by a lower limit of about 0.01% below which effective anti-rusting properties are not obtained, and an upper limit in the neighborhood of 0.10% above which the emulsion problem becomes too severe for commercial practicability. The preferred quantity of the degras fatty acids for the purpose of this invention is of the order of 0.03%.

Broadly, this invention contemplates the incorporation, in the aforesaid turbine oil, of degras fatty acids which are obtained from degras, a mixture of fatty acids, fatty alcohols and fatty esters. Degras fatty acids may be prepared from degras by various means, and may be purchased on the market. The fatty acids vary in neutralization number and it is believed that such variation is associated with the method of preparation and may or may not be associated with differences in degras itself. For example, typical degras fatty acids were prepared in the following ways.

## EXAMPLE I

A specimen of wool grease was saponified under

pressure with alcoholic potassium hydroxide. The unsaponifiable material (fatty alcohols and fatty esters) was removed from the soap mixture formed in the saponification step, with solvent. The fatty acids were recovered by acidifying the soap solution with mineral acid and extracting with solvent. The fatty acids thus obtained were free of mineral acids and solvent, and had a neutralization number (N. N.) of 163.

#### EXAMPLE II

A specimen of wool grease was saponified under pressure with alcoholic potassium hydroxide and with methyl ethyl ketone as a solvent. The unsaponifiable material was removed with solvents, the fatty acids were recovered from the soap solution with a solvent after acidification, and the solvent was subsequently removed from the fatty acids. The fatty acids so obtained were free of mineral acid and solvent, and had a neutralization number ranging from 86 to 147. The fatty acids of lower N. N., from 86 to 110, were less effective in turbine oils than were those of higher N. N., from 110 to 147. For example, 0.02% to 0.03% of the fatty acids having an N. N. of from 110 to 147 gave perfect rust tests (described below); whereas, those fatty acids having an N. N. of from 86 to 110, while effective anti-rusting agents, were required in larger amounts to produce good results.

All degras fatty acids are effective for the purposes of this invention, and particularly effective—and preferred—are those fatty acids obtained from degras which have a neutralization number of from about 110 to about 170.

In combination with the degras fatty acids in the aforesaid turbine oils is an aniline disulphide, that is aniline disulphide itself or an alkyl-substituted aniline disulphide, which functions as an antioxidant. The aniline disulphides contemplated herein may be represented by the general formula:



wherein, R and R' are selected from the group consisting of hydrogen and alkyl radicals.

The oil used in the composition hereinbefore described may be of the type normally used for the lubrication of steam turbines. In general, the oil may be defined as a viscous mineral oil fraction having a Saybolt Universal viscosity of from 100 to 600 seconds at 100° F. Typical turbine oils with which a mixture of an aniline disulphide and degras fatty acids have been admixed to provide improved turbine oils have the following specifications:

Table I

|                       | Oil A   | Oil B |
|-----------------------|---------|-------|
| Gravity, °A. P. I.    | 28.4    | 22.3  |
| Pour Test, °F.        | 5       | -10   |
| Flash, °F.            | 385     | 420   |
| Color, A. S. T. M.    | 1       | 2½    |
| Viscosity, Saybolt at |         |       |
| 100° F.               | 148-155 | 681   |
| 130° F.               | 84.5    | 259.5 |
| 210° F.               | 43      | 61.2  |

To demonstrate the efficacy of the combination of an aniline disulphide and degras fatty acids in turbine oils, typical turbine oil compositions comprising oils A and B and very small amounts

of aniline disulphide and representative degras fatty acids were tested in the following manner.

Polished steel specimens were suspended in the oil compositions and water and heated to a predetermined temperature for a predetermined time. In some instances, as will appear from the table below, the temperature was 140° F. and in others it was 167° F.; also, as will appear from the table, the time interval was 24 hours in some of the tests and in others it was 48 hours. The mixture was agitated constantly by a motor driven stirrer. The improving agents used in the oil samples tested are indicated by the abbreviations A. D. S. (aniline disulphide) and D. F. A. (degras fatty acids). The neutralization number (N. N.) of the degras fatty acid used is also indicated.

Table II

|    | Oil | Improving agent | Per cent | Per cent water | Temp., °F. | Time, hrs. | Condition of steel specimens |
|----|-----|-----------------|----------|----------------|------------|------------|------------------------------|
| 20 | A   | None            |          | 1.0            | 140        | 24         | Rust.                        |
|    | A   | A. D. S.        | 0.1      | 1.0            | 140        | 24         | Do.                          |
|    | A   | A. D. S.        | 0.1      | 1.0            | 140        | 24         | No rust.                     |
| 25 | A   | D. F. A.        | 0.1      |                |            |            |                              |
|    | A   | (N. N. = 163)   |          |                |            |            |                              |
|    | A   | A. D. S.        | 0.1      | 1.0            | 140        | 24         | Do.                          |
|    | A   | D. F. A.        | 0.02     |                |            |            |                              |
|    | A   | (N. N. = 163)   |          |                |            |            |                              |
| 30 | A   | A. D. S.        | 0.1      | 10.0           | 167        | 48         | Do.                          |
|    | A   | D. F. A.        | 0.02     |                |            |            |                              |
|    | A   | (N. N. = 163)   |          |                |            |            |                              |
|    | A   | A. D. S.        | 0.1      | 10.0           | 167        | (24)       | Do.                          |
|    | A   | D. F. A.        | 0.01     |                |            | (48)       | Do.                          |
| 35 | B   | None            |          | 10.0           | 167        | 48         | Rust.                        |
|    | B   | A. D. S.        | 0.1      | 10.0           | 167        | 48         | Do.                          |
|    | B   | A. D. S.        | 0.1      | 10.0           | 167        | 48         | No rust.                     |
|    | B   | D. F. A.        | 0.03     |                |            |            |                              |
|    | B   | (N. N. = 130)   |          |                |            |            |                              |

The effectiveness of the combination of aniline disulphide and degras fatty acids to inhibit the deleterious effects of oxidation upon turbine oils is shown by the results of the following Brown-Boveri oxidation tests tabulated below in Table III. A typical turbine oil composition, as contemplated by the present invention, comprising oil A, 0.1% of aniline disulphide and 0.02% of degras fatty acids (N. N. = 163) was compared with an oil composition comprising oil A and 0.1% of aniline disulphide. That the oxidation characteristics of the oil were only slightly changed by the addition of degras fatty acids is evident from the results given in Table III.

Table III

|    | Oil | Improving agent | Per cent | Color Lovibond | N. N. | Sludge |
|----|-----|-----------------|----------|----------------|-------|--------|
| 55 | A   | A. D. S.        | 0.1      |                | 15    | 0.03   |
|    | A   | A. D. S.        | 0.1      |                | 24    | 0.05   |
|    | A   | D. F. A.        | 0.02     |                |       |        |
|    | A   | (N. N. = 163)   |          |                |       |        |
| 60 |     |                 |          |                |       |        |

From the foregoing it will be seen that minor proportions of an aniline disulphide and degras fatty acids in turbine oils will provide lubricants which may be used effectively in the presence of moisture to prevent rusting of ferrous metal parts by the moisture present, and to prevent changes in the oxidation characteristics of such oils in such an environment. It is to be understood that although we have herein described and illustrated the invention with certain preferred mineral oil blends, the invention is not restricted to the specific examples given but includes within its scope whatever changes fairly come within the spirit of the appended claims.

I claim:

1. An oil composition adapted for the lubrication of ferrous metal surfaces in an environment containing water, comprising a viscous mineral oil having in admixture therewith a minor proportion, from about 0.01% to about 0.1%, of degras fatty acids and a minor proportion, from about 0.05% to about 0.2%, of a compound selected from the group consisting of aniline disulphide and alkyl-substituted aniline disulphides.

2. An oil composition adapted for the lubrication of ferrous metal surfaces in an environment containing water, comprising a viscous mineral oil having in admixture therewith a minor proportion, about 0.03%, of degras fatty acids and a minor proportion, from about 0.05% to about 0.2%, of a compound selected from the group consisting of aniline disulphide and alkyl-substituted aniline disulphides.

3. An oil composition adapted for the lubrication of ferrous metal surfaces in an environment containing water, comprising a viscous mineral oil having in admixture therewith a minor proportion, from about 0.01% to about 0.1%, of degras fatty acids having a neutralization number of from about 110 to 170, and a minor proportion, from about 0.05% to about 0.2%, of a compound selected from the group

consisting of aniline disulphide and alkyl-substituted aniline disulphides.

4. An oil composition adapted for the lubrication of ferrous metal surfaces in an environment containing water, comprising a viscous mineral oil having in admixture therewith a minor proportion, from about 0.01% to about 0.1%, of degras fatty acids having a neutralization number of from about 110 to about 170, and a minor proportion, from about 0.05% to about 0.2%, of aniline disulphide.

5. A turbine oil composition comprising a mineral oil fraction having a Saybolt Universal viscosity of from 100 seconds to 600 seconds at 100° F. and having in admixture therewith a minor proportion, from about 0.01% to about 0.1%, of degras fatty acids and a minor proportion, from about 0.05% to about 0.2%, of a compound selected from the group consisting of aniline disulphide and alkyl-substituted aniline disulphides.

6. An oil composition adapted for the lubrication of ferrous metal surfaces in an environment containing water, comprising a viscous mineral oil having in admixture therewith about 0.03% of degras fatty acids and about 0.1% of aniline disulfide.

JOHN H. BISHOP.